

# United States Patent Office

2,702,266

Patented Feb. 15, 1955

1

2,702,266

## BRIQUETTING ASPHALT COMPOSITION AND PROCESS OF MAKING SAME

Mathew L. Kalinowski, Chicago, Ill., assignor to Standard Oil Company, Chicago, Ill., a corporation of Indiana

No Drawing. Application February 27, 1951,  
Serial No. 213,055

4 Claims. (Cl. 196—22)

This invention relates to an improved asphalt composition and to the method of its manufacture. The invention refers particularly to asphalt compositions having increased compressive and cohesive strength, and, because of this increased strength, greater suitability for briquetting purposes.

The widespread employment of cracking processes in petroleum refining supplies a large volume of asphaltic residues which yield asphalts that are useful as binding agents in aggregate compositions, an important one of which is solid-fuel briquettes. However, these cracked petroleum asphalts as a class are often too brittle or in some other strength characteristic do not meet specifications defining briquetting agents of suitable binding strength. A primary object of the present invention is therefore the provision of an asphalt composition having improved strength characteristics. Another object of the invention is the provision of a method of preparing improved asphalt compositions. Yet another object of invention is the provision of an improved briquetting asphalt.

I have found that the foregoing objects can be accomplished by the incorporation in the asphalt of the treated by-product of a well-known process of chemical petroleum refining of lubricating oils. In this chemical-refining process, lubricating oils, which may previously have been dewaxed, are extracted with phenol or phenol homologs to remove undesirable constituents. The extraction of these constituents, which include petroleum resins and aromatic compounds, results in increasing the viscosity index of the oils as well as effecting other improvements. The phenolic solvent can be recovered from the extract by any one of several known methods including, for example, steam distillation. The phenol-free, undesirable constituents of lubricating oils, obtained by the phenol extraction process described briefly above, are hereinafter referred to as "phenol extract."

Briefly stated, the present invention comprises the method of, and the asphalt composition provided by, extracting a phenol extract of a lubricating oil with a hydrocarbon solvent consisting of one or more paraffinic hydrocarbons having more than one and less than about eight carbon atoms per molecule and being preferably a normally gaseous hydrocarbon, thereafter separating a resinous, raffinate phase and extract oils phase, removing solvent from the resinous raffinate phase, and incorporating in preferably a cracked-petroleum asphalt from about 5 to 25 percent, by weight based on the asphalt, of solvent free resins from the said raffinate phase. Compositions containing any petroleum asphalt and an amount, within the said range, of the extract resins will provide suitable briquetting asphalts. However, the invention is especially applicable to cracked-petroleum asphalts and to improving the strength characteristics of these asphalts for use as binding agents. Cracked-petroleum asphalts are obtained by the reduction of tars from cracking processes. These asphalts are usually air-blown at elevated temperatures to a softening point of between about 150° and 200° F. The said solvent-free resins constitute primarily petroleum resins characterized by a melting point between about 80° and 120° F., a specific gravity between about 0.85 and 0.95 at 77° F., and a color as determined by the ASTM method 115—45T of about 8. The raffinate will also contain minor quantities, at most about 35 percent, of wax-like material as determined by ASTM method D—721—47; this method may report as wax some of the aforementioned resins. This minor content of waxy material will,

2

of course, be substantially eliminated when the lubricating oils are dewaxed before extraction with phenol.

In the preparation of the said phenol extract, a distillate oil is obtained by the distillation in fractionating equipment of a reduced crude petroleum. The reduced crude can be fractionated, for example, into such lubricating oil types as SAE 10, 20 or 40. This oil is usually not dewaxed before phenol extraction because sufficiently high temperatures are employed during extraction to prevent precipitation of the wax during the extraction step. The phenol extraction is preferably carried out in a countercurrent multi-stage operation equivalent to about five to seven stages using from 2 to 4 volumes of phenol for each volume of oil and employing temperatures between about 160°—180° F. at the top of the extraction tower and 140°—160° F. at the bottom thereof. Water is preferably injected into the extraction mixture near the bottom of the tower to improve the selectivity of the phenol extractant. The degree of extraction obtained is directly reflected in the viscosity index of the treated oil, more intense treatment resulting in higher viscosity indexes. The phenol can be removed from the extract by any of the known solvent reclaiming methods and preferably by the method of fractional distillation and steam stripping described and claimed in Sullivan U. S. 2,111,822 patented March 22, 1938.

The phenol extract, that is obtained by separation of the phenolic solvent from the extract, is then treated according to the hereinafter described method with a hydrocarbon solvent consisting of one or more paraffinic hydrocarbons having less than about eight carbon atoms per molecule, or between two and seven carbon atoms per molecule, inclusive, and preferably with a lower molecular weight hydrocarbon within this class.

When a normally gaseous hydrocarbon such as propane is used as the hydrocarbon extractant, the phenol extract is treated under propane deresining conditions. For example, propane and phenol extract are mixed at about 100° F. in a ratio of about 8 volumes of propane for each volume of phenol extract, the mixture is then heated to a temperature in the range of about 140° F. to 190° F., at which temperature autogenic pressure is about 350 pounds per square inch and separate phases of propane extract and propane raffinate are formed. The propane extract and propane raffinate are separated, propane is stripped from the heavier raffinate phase, and the remaining extracted resinous material constitutes the additive employed in the present invention.

When a normally liquid hydrocarbon is employed the phenol extract and the hydrocarbon are preferably separately cooled to a temperature below about 0° F., preferably between about —60° F. and —20° F., and, when hexane is employed as extracting solvent, to preferably about —40° F. The phenol extract and hexane are then introduced into an extraction zone in a proportion of about 2 to 10 volumes of hydrocarbon per volume of phenol extract. By an alternate method, the phenol extract and normally liquid extractant can be mixed before the cooling step, in which case they form a single mutually miscible solution. When cooled to a temperature of between —60° F. to —20° F. the solution forms a two phase system. When adequate extraction and settling is obtained, separation can be accomplished by siphoning off the supernatant extract phase.

Propane and phenol extract, which have been separately introduced into a vertically extending extraction zone, are passed counter-currently through the said zone and will be separated one from the other in settling zones at the opposite ends of the extraction zone. The propane extract that is removed from the top of the extraction zone is then stripped of propane by releasing the pressure. The recycled propane is cooled, condensed and can be recycled to the extract step. The extract remaining after removal of the propane consists of the oil components of the treated phenol extract, which components usually comprise about 70 percent by weight of the total phenol extract.

The propane raffinate that is separated by either decanting the propane extract from the surface of the liquid or by the above described countercurrent operation is stripped of propane by release of pressure, the propane that is dis-

solved in the raffinate solution being permitted to escape therefrom. The released propane can be cooled, condensed, and recycled to further extraction.

The reduced raffinate contains the said petroleum resins and a minor quantity of wax. Yields of resins ranging from about 10 to 40 percent by weight of the phenol extract have been obtained.

Pressure-still asphalt and about 2 to 25 percent by weight of the phenol-extract resins are thoroughly mixed at a temperature between about 200° and 400° F. and at 10 preferably about 300° F. Coal briquets consisting of coal fines and a small amount, preferably between 4 to 8 percent by weight, of the asphalt briquetting composition show good strength and stability.

It has been found that the total phenol extract is not effective as an additive to provide a briquetting asphalt, and that asphalts incorporating the total extract are not satisfactory briquetting agents. The light-hydrocarbon-insoluble resinous fraction of the phenol extract is, on the other hand, effective to improve the binding characteristics of asphalt as demonstrated in the following specific examples.

#### EXAMPLE I

Lubricating oils in the three grades SAE 10, 20 and 40 were obtained by distilling, under vacuum, a reduced Mid-Continental crude oil from which 62 percent of the lighter ends had previously been removed. These distillate oils contained wax to the extent of 5 weight percent for the SAE 10 distillate to about 9 weight percent for the SAE 40 distillate.

The three lubricating oils were each treated with a phenol extractant in a countercurrent multi-stage operation in which about 2.5 volumes of phenol were used for each volume of oil. The temperature of the extraction mixture was about 160° to 180° F. at the top of the extraction tower and about 140° to 160° F. at the bottom thereof. Water in the amount of 5 weight percent of the phenol was injected near the bottom of the tower to improve the selectivity of the phenol for undesirable components of the lubricating oil. Operation of the extraction unit was adjusted carefully to obtain certain viscosity indexes for each grade of oil. The phenol was substantially entirely removed from the phenol extract by first flashing phenol from the extract material and then steam stripping to remove the remaining phenol from the extract. The yields of phenol extract ranged between about 40 and 45 percent.

About one part of phenol extract from each of the distillate oils was each dissolved in five parts of hexane and the solutions were cooled to about -40° F. At this temperature a two phase system was formed and separation was effected by siphoning off the supernatant extraction phase. This hexane extraction accomplished a distribution of the phenol extract in the proportion of about 30 percent as resinous components in the raffinate phase and about 70 percent as oils in the supernatant extract phase. After separation of the phases and subsequent removal of hexane by flash distillation of this light solvent from the raffinate phase, the resin fraction of a phenol extract was obtained. There were obtained from the said lubricating oils, SAE 10, 20 and 40, resin yields respectively, of 31, 10 and 20 weight percent. These phenol extract resins exhibited the properties outlined in the following table:

Table I.—Physical properties of phenol extract resins

| Resin from            | Melting Point<br>ASTM<br>D87-42,<br>° F. | Sp. Gr.,<br>77° F. | Color<br>NPA<br>ASTM<br>155-45T |
|-----------------------|------------------------------------------|--------------------|---------------------------------|
| SAE 10 Phenol Extract | 86                                       | 0.90               | 8+                              |
| SAE 20 Phenol Extract | 115                                      | 0.88               | 8+                              |
| SAE 40 Phenol Extract | 116                                      | 0.87               | 8+                              |

A briquetting asphalt composition was prepared by blending an asphalt, obtained by reducing and oxidizing a cracked tar to a softening point of 170° F., with 18 percent by weight based on the asphalt of the above prepared resin fraction of phenol extract of SAE 10 lubricating oil. This composition was prepared by heating and stirring asphalt at a temperature of about 300° F. while adding the described resin component. The asphalt was

also blended with 25 percent by weight of each of the resin extracts of SAE 20 and SAE 40 oils.

5 A portion of the total phenol extract (without hydrocarbon solvent extraction) from SAE 10 oil, equal in weight to the above employed weight of resin extract from SAE 10, was added to a proportionate weight of the same asphalt and mixed therewith at the same temperature. The total phenol extracts of the other oils were also blended with samples of the same asphalt at the same temperature.

10 Briquetting asphalts consisting of the untreated asphalt and compositions containing 18% of the total phenol extract in some cases and 18% of the extract resins in others were mixed with fine coal in the amount of 6% by weight of asphalt based on the weight of the coal, and the mixtures were briquetted under standardized conditions. The so-formed briquets were tested for compressive strength as reported in Table 2.

15 As shown in this table in which the effect of total phenol extract and the resin extract from phenol extract of an SAE 10 lubricating oil are compared, the total phenol extracts were ineffective as additives to provide a suitable briquetting asphalt.

Table 2.—Effect on asphalt physical properties of phenol extract resin compared to total phenol extract

|    | Untreated Asphalt                                    | Asphalt +18% Phenol Extract Resins | Asphalt +18% Total Phenol Extract | Briquetting Asphalt Requirements |
|----|------------------------------------------------------|------------------------------------|-----------------------------------|----------------------------------|
| 30 |                                                      |                                    |                                   |                                  |
| 35 | Softening Point, ° F.                                | 175.....                           | 135                               | 135 130-140.                     |
|    | Penetration at 77° F.                                | 2.....                             | 18                                | 19 Between 15-20.                |
| 40 | Ductility at 77° F. <sup>1</sup>                     | Shatters.....                      | 100+ 1.07                         | .18 min. 100.                    |
|    | Specific Gravity                                     | 1.13.....                          | 1.07                              | 1.09 min. 106.                   |
|    | Flash, ° F., C. O. C.                                | 565.....                           | 500                               | 495 min. 450.                    |
|    | Cohesive Strength of Asphalt (p. s. i.) <sup>2</sup> | Shatters.....                      | 100                               | 71 min. 85.                      |
| 45 | Compressive Strength (Lbs.) <sup>3</sup>             | 135.....                           | 225                               | 181 min. 200.                    |

<sup>1</sup> Ductility as determined by ASTM test D 113-44.

<sup>2</sup> Cohesive strength is a pressure required to shear a strip of asphalt one-half inch wide by one inch long and 0.010 inch  $\pm$  0.002 inch thick at a uniform rate of shear in a Perkin's tensile tester manufactured by B. F. Perkins and Son, Inc. of Holyoke, Mass.

<sup>3</sup> Compressive strength is determined with a Komarek-Greaves compression tester. The test is made on a coal briquet consisting of coal fines and 6% of briquetting asphalt. Compressive strength is the force required to crush a coal briquet at 80° F.

50 It is to be observed in the above table that the asphalt compositions containing resin extracts in every case meet all the requirements of the briquetting asphalt specifications listed in the above table. It is further noted that the employment of the total phenol extract while lowering the softening point and increasing the penetration to the required extent failed to increase ductility, cohesive or compressive strength to a degree needed to provide an acceptable briquetting asphalt. The improvement provided by the extract resins was obtained without so altering the characteristics of the asphalt as to render it, in some other respect, unsuitable for coal briquetting. This characteristic of the extract resins is important because, while it might be expected that many oils could be blended with brittle asphalt to plasticize it, such additives degrade strength characteristics and otherwise alter the asphalt and render it unacceptable for binding purposes.

#### EXAMPLE II

75 The resin fraction of the phenol extract of an SAE 10 lubricating oil was obtained by mixing one part of the extract with five parts of hexane and cooling the solution that formed to -40° F. A two phase system was formed and separation was effected by siphoning off the supernatant extract phase. After removal of the hexane by evaporation, the desired resinous components were recovered in about 31 percent yield based on the employed weight of phenol extract.

80 A cracked-petroleum asphalt having a softening point of 170° F. was blended with 18 percent by weight of the resin fraction of phenol extract by heating and stirring the two components at 300° F. In a similar manner, another portion of the same asphalt was blended with 18 percent of the untreated total phenol extract. When the

untreated asphalt is subjected to the cohesive strength test described in Example I, it shatters. The asphalt composition containing the resin extract exhibited a cohesive strength of 100 pounds per square inch while the asphalt composition containing the total phenol extract had a cohesive strength of only 60 pounds per square inch.

### EXAMPLE III

When employing propane instead of hexane as a solvent, one part of a phenol extract of a lubricating oil is dissolved in 8 parts of propane under a pressure of about 350 pounds per square inch and at a temperature of about 150° F. At this temperature a two phase liquid system is formed, a supernatant extract phase containing oils from the phenol extract and a raffinate phase consisting of solvent and, predominantly, resins. The phases are separated by decanting the upper layer from the pressure vessel, and propane is removed from the lower resinous layer by releasing the product to atmospheric pressure. A briquetting asphalt having suitable ductility and cohesive and compressive strength can be prepared by mixing about 20% by weight of the said resin with a pressure still asphalt and heating and stirring the said admixture at 300° F.

The improved asphalt composition provided by the present invention has been described primarily as a briquetting asphalt but of course the improved characteristics of the composition render it especially suitable for other binding purposes, and for use, for example, in floor tile or road making compositions.

Having described my invention, I claim:

1. An asphalt composition comprising a cracked-petroleum asphalt and a small amount of a resinous product that is obtained by the steps of extracting a distillate lubricating oil with a phenolic type extractant, separating the phenolic extract from the treated lubricating oil, stripping the phenolic extractant from the said extract, admixing the said extract and a paraffinic hydrocarbon containing less than eight carbon atoms per molecule, subjecting the mixture to a temperature at which it forms two separate liquid phases, one consisting of an oily portion of the said phenolic extract in solution in the hydrocarbon and another containing the resinous portion of the phenolic extract, separating the said liquid phases, removing hydrocarbon solvent from the so-separated resinous portion of the phenolic extract, and recovering the said resinous product therefrom.

2. The composition of claim 1 in which the amount of resinous product is in the range of about 5 percent to about 25 percent by weight, based on the asphalt.

3. A method of preparing an asphalt composition suitable for briquetting, the said method comprising admixing an asphalt, that is obtained from the tarry residue of a cracking of reduced-crude petroleum, with from 5 to 25 percent, by weight of the said asphalt, of a resinous product that is obtained by the steps of extracting a distillate lubricating oil with a phenolic type extractant, separating the phenolic extractant from the treated lubricating oil, stripping the phenolic extractant from the said extract, admixing the said extract and a paraffinic hydrocarbon containing less than eight carbon atoms per molecule, subjecting the mixture to a temperature at which it forms two separate liquid phases, one consisting of an oily portion of the said phenolic extract in solution in the hydrocarbon and another containing the resinous portion of said phenolic extract, separating the said liquid phases, removing hydrocarbon solvent from the so-separated resinous portion of the phenolic extract and recovering therefrom the said resinous product, and heating the said asphalt and the resinous product to a temperature of between about 200° and 400° F. while stirring to obtain thorough mixing.

4. A method of preparing an asphalt composition that is suitable for briquetting, the said method comprising admixing from two to ten volumes of a paraffinic hydrocarbon having more than two and less than about eight carbon atoms per molecule with one volume of a phenol extract of a distillate lubricating oil from which extract the phenol has been stripped, subjecting the admixture to a temperature at which it forms an extract oils phase and a resinous raffinate phase, separating the resinous phase from the oils phase, removing hydrocarbon solvent from the resinous phase, mixing a cracked-petroleum asphalt and from two to twenty-five percent, by weight based on the asphalt, of solvent-free resins, heating the asphalt and resins and mixing the same at a temperature between about 200° and 400° F.

### References Cited in the file of this patent

#### UNITED STATES PATENTS

|           |                  |       |               |
|-----------|------------------|-------|---------------|
| 1,987,085 | Thurston         | ----- | Jan. 8, 1935  |
| 1,989,045 | Merrill          | ----- | Jan. 22, 1935 |
| 1,993,532 | Skowronski       | ----- | Mar. 5, 1935  |
| 2,024,096 | Dengler et al.   | ----- | Dec. 10, 1935 |
| 2,120,376 | Shipp et al.     | ----- | June 14, 1938 |
| 2,317,150 | Lovell et al.    | ----- | Apr. 20, 1943 |
| 2,455,709 | Spelhouse et al. | ----- | Dec. 7, 1948  |